

## UNITED STATES PATENT OFFICE

2,318,296

## ANTISTATIC AGENT AND ITS APPLICATION

Joseph B. Dickey, Rochester, N. Y., assignor to  
Eastman Kodak Company, Rochester, N. Y., a  
corporation of New Jersey

No Drawing. Application December 23, 1940,  
Serial No. 371,402

12 Claims. (Cl. 8—142.5)

This invention relates to the treatment of cellulose organic derivative filaments, fibers, threads and the like and more particularly to a method of eliminating the tendency of such materials to accumulate charges of static electricity in twisting, winding and spinning. The invention also relates particularly to the treatment of cellulose organic derivative cut staple fibers to adapt them for the manufacture of spun yarns.

As is well-known, cellulose organic derivative materials, particularly in filament, yarn, or sheet form, are particularly subject to the accumulation on their surfaces of charges of static electricity from frictional and other influences. In the case of filaments and yarns in which the surface area of the material (per unit of weight) is enormously greater as compared to sheets or films, the problem of static often assumes serious proportions. In the manufacture of yarns of various types from artificial filaments, numerous steps in which the yarn is subjected to frictional influences may be necessary, as for example, twisting, winding, warping, carding, combing, drawing, spinning and the like, all of which operations tend to produce large accumulations of static on the filaments. This is particularly aggravated in the utilization of cut staple, as for example, in the making of spun yarn, since in carding and combing considerable friction is developed and as a result sufficient charges accumulate on the fibers to make the formation of the web difficult, if not impossible; furthermore, even if a web is formed with some degree of success, the subsequent drafting operation produces a very uneven spun yarn or intermediate roving due to the presence of the static charge. In addition, there is the ever-present fire hazard.

Cellulose derivative yarn, particularly in the form of cut staple, is extremely difficult to handle in the various operations involved in making spun yarn, not only because such material is composed of filaments having smooth, glass-like surfaces without natural kink or irregularity, but also because it has relatively negligible moisture content at normal humidities, as compared to natural fibers such as cotton and wool, making it inherently far more susceptible to the accumulation of static. The charges accumulating on cellulose derivative cut staple fibers, are, under some cir-

cumstances, even sufficient to separate the individual fibers a distance of inches, notwithstanding their relatively minute size.

This invention has as its principal object to provide an improved method for the treatment of cellulose organic derivative yarns to reduce or eliminate the tendency of such yarns to accumulate charges of electricity under frictional and other influences. A further object is to provide a method of facilitating the handling and employment of cellulose organic derivative cut staple fibers in the various operations involved in the manufacture of spun yarns. A still further object is to provide a method of treating cellulose organic derivative yarns in either filament or cut staple form, wherein the material is simultaneously softened and lubricated and the accumulation of static charges thereon is prevented. Another object is to provide an improved type of cellulose organic derivative cut staple having little or no tendency toward accumulation of static electrical charges. Other objects will appear hereinafter.

These objects are accomplished by the following invention which, in its broader aspects, comprises applying to cellulose organic derivative yarns either in the form of filaments, threads, or staple fibers, an antistatic composition characterized by the presence therein of phosphoric, phosphorus, and sulfuric acid esters of alcohols having the general formula:



wherein R is an alkyl radical selected from the group consisting of methyl, ethyl, butyl, amyl, hexyl, cyclohexyl, allyl, octyl, lauryl, cetyl, oleyl, hydroxy ethyl, naphthyl, tetrahydrofurfuryl, decahydronaphthol, triethylene glycol, Carbitol (the trade name for the monoethyl ether of diethylene glycol), etc., and x is 0, 1, 2, etc., and Z is a mono-valent substituent selected from the group consisting of alkyl, hydroxyl, aryl and the like.



of the types indicated in Example 1 may be prepared. Various amide derivatives may be prepared by treating the acid chloride with ammonia. Thus,



(2-hexylcyclohexyl phosphamate sodium salt)



(2-laurylcyclohexyl bisbutyl phosphamate)



(2-naphthylcyclohexyl thio-phosphate morphamite ammonium salt)

**Example 7**

204 g. 2-beta-phenylethyl cyclohexanol are dissolved in pyridine and phosphated with 163 g. C<sub>2</sub>H<sub>5</sub>OPOCl<sub>2</sub> by adding the acid chloride and warming to 50°. The acid chloride is hydrolyzed and the desired salt prepared as in Example 6. In a similar way we may prepare:



(2-tetrahydrofuryl cyclohexyl phosphate mono-beta-ethoxy ester)



(4-cetyl cyclohexyl thio-phosphate mono-methyl ester mono-potassium salt)

**Example 8**

156 g. 2-butylcyclohexanol are heated in dioxane with one equivalent of P<sub>2</sub>O<sub>5</sub> at 100° for 6 hours. The product has the formula:



(2-butyl cyclohexyl phosphate)

In a similar way



(4-butyl cyclohexyl thiophosphate)

may be prepared.

**Example 9**

One mole 2-butylcyclohexanol is treated with one mole PCl<sub>3</sub> and warmed to complete the reaction. The resulting dichloride, after evacuation to remove hydrogen chloride, is then treated

with cold aqueous sodium carbonate, and the compound



(2-butyl cyclohexyl disodium phosphite)

is formed.

10 By neutralizing the salt with mineral acid and then treating with the desired base, any desired organic base salt can be prepared.

**Example 10**

15 One mole of



20

is heated on a water bath with one mole of pyridine to give



(2-butyl cyclohexyl sulfonyl pyridinium chloride)

40 Compounds of this type are particularly useful as antistatic agents, soap, wetting agents, etc. In place of pyridine we may use tributylamine, ethyl piperidine, diethylcyclohexylamine, etc.

**Example 11**

45 One mole 2-cetyl-4-isobutyl cyclohexanol is reacted with one mole phosphorous trichloride as previously described. The acid chloride is hydrolyzed with 1.5 moles sodium carbonate and the 2-cetyl-4-isobutyl cyclohexyl phosphorous acid is filtered off. Any desired salt as indicated in the previous examples can be prepared. Similarly, there may be prepared compounds such as 2-oleyl cyclohexyl phosphite, 2,4,6-tri-isopropyl 55 cyclohexyl phosphite, 2,4-di-isobutyl cyclohexyl phosphite and 2-beta-ethoxy-beta-ethoxy ethyl cyclohexyl phosphite, etc.

In like manner, pyrophosphoric acid or tetraphyrophosphoric acid may be used as phosphating agents in a manner similar to the use of the phosphating and phosphiting agents referred to in the above examples.

60 In accordance with my invention the above-mentioned compounds may be applied to the yarn in any convenient manner, for example, by roll, wick, immersion, spraying or the like. Inasmuch as these compounds are soluble in oil they may be dissolved or dispersed in oils such as mineral oil, blown and unblown, drying and semi-drying. 70 vegetable and animal oils, examples of which are light mineral, neat's-foot, olive, teased, castor, soya bean, rapeseed oils and other lubricants, etc.

65 In the following examples and description, I have set forth several of the preferred embodiment

ments of my invention, but they are included merely for purposes of illustration and not as a limitation thereof.

*Example 12*



(2-butyl cyclohexanol phosphate bis-diethylcyclohexylamine salt)

is applied to textile materials (silk, cotton, wool, viscose, cellulose acetate, etc.) by means of a wick, roller, spray, etc., to facilitate their knitting, weaving, spinning and the like. Yarns lubricated with the above types of lubricants are of special value in the preparation of cut staple fibers. These fibers may be oiled before or after cutting.

*Example 13*



(2-amyl-4-methyl cyclohexanol sulfate ditetrahydrofurfurylamine salt)

Conditioning liquids particularly useful for the treatment of various types of yarns in accordance with my invention particularly those composed of or containing cellulose acetate, cellulose acetate propionate, cellulose acetate butyrate, and similar organic acid esters, and especially adapted for the deelectrification or anti-static treatment of cellulose organic derivative cut staple yarns are as follows:

*Example 14*

Parts  
Dioxane dioleyl ether----- 80  
 $\beta, \beta'$ -tetrahydrofurfuryloxyethyl ether----- 10



(2-hexylcyclohexanol phosphate monoethyl ester sodium salt)

Water----- 5

and applied to textile materials such as silk, wool, cellulose acetate, etc., as described in Example 12. If the yarn is intended primarily for knitting, the amount of conditioning liquid applied may vary from 4-25 per cent by weight of the yarn and if for weaving, between 1-5 per cent by weight.

Cellulose acetate filaments treated as described above are quite soft and pliable and give improved results in various textile operations such as weaving, knitting, etc., and especially in the production of cut staple yarn. Other examples of suitable lubricating mixtures having antistatic properties which are used as illustrated in Examples 12 and 13 follow:

*Example 15*

A conditioning liquid particularly useful on cut

staple fibers made of cellulose acetate and which may be used for other textile operations follows:

Parts



(2-benzyl cyclohexanol phosphate bis-diethylamine salt)

5  
95

Olive oil-----

*Example 16*



(2-hexyl-p-methyl cyclohexanol-sulfate naphthylamine salt)

Parts

5  
30-70  
Blown olive oil----- 65-25

*Example 17*



5  
30-50  
35 (2-lauryl cyclohexanol phosphite diethyl-cyclohexylamine salt)

Neat's-foot oil-----

Parts

5  
95

*Example 18*



(2-octyl cyclohexanol thiosulfate morpholine salt)

Parts

5  
95

Blown neat's-foot oil-----

5  
95

*Example 19*



5  
30-50  
55 (2-hexyl cyclohexanol sulfate diethyl cyclohexylamine salt)

Parts

5  
10

Mineral oil-----

30

Blown olive oil----- 65-60

*Example 20*



5  
65-70  
65 (2-tetrahydrofurfuryl cyclohexanol thiophosphate butylamide benzyl trimethyl ammonium hydroxide salt)

Parts

5  
10

Sperm oil-----

65

75 Tetrahydrofurfuryl lactate----- 30

## Example 21

Parts



(2-hexyl-m-butyl-p-hydroxy-cyclohexanol phosphate tetrahydrofurylamine dicyclohexylamine salt)

Blown olive oil

5

Blown sperm oil ----- 5  
Mineral oil ----- 60

## Example 22

Parts

Di-beta-methoxy ethyl succinate ----- 30



(2-allyl cyclohexanol sulfate triethanolamine triacetate salt)

Teased oil ----- 1-10  
64-55

## Example 23

Parts

Mineral oil ----- 90-99



(2-sodium-beta-phosphito-beta-ethoxy-beta-ethoxy ethyl cyclohexyl phosphite diethanolamine salt)

1-10

## Example 24

Parts



(2-octadecyl cyclohexanol sulfate di-beta-methoxy ethylamine salt)

Oleic acid ----- 5  
20



Sodium sulfate ----- 5  
Blown teased oil ----- 2

5

68

Water ----- 70  
Water soluble cellulose ester ----- 15

70

15



(2-beta-morpholino ethyl cyclohexanol phosphite)

Sulfonated castor oil ----- 5  
10

5

75

## Example 26

Parts

80-99



(2-allyl cyclohexanol disodium phosphate)

20-1

## Example 27

Parts



(2-butyl cyclohexanol phosphite diethyl cyclohexylamine salt)

1-15

Any of the above compositions may be applied to the yarn intended for use in circular knitting by means of a bath, wick, spray, roller, pad or any suitable means. The amount of conditioning liquid applied may vary between 5-25% by weight of the yarn. Usually, however, the amount of conditioning liquid applied is about 10-15% by weight of the yarn. Yarn composed of cellulose acetate conditioned as described above gives excellent results when used in the circular knitting process.

As will be apparent from the above examples and description the conditioning agents of my invention may be applied by a wide variety of methods. For example, we may employ the agent as an ingredient of the spinning dope from which filaments are formed, the amount of the agent so employed depending upon a number of factors, such as the particular cellulose derivative used in making the yarn, the solvent or solvent combination used in making up the spinning solution, and properties desired in the finished yarn, etc.

If the conditioning agent is to be applied to the yarn after spinning, this may be done by bringing the yarn in contact with a wick, roll, or felt wet therewith, or the liquid may be applied by immersion, spray, or otherwise. The particular point at which the liquid is applied may vary. It may, for example, be applied to the yarn inside or outside the spinning cabinet, between the guide and godet roll, between the godet or other roll or guide and the point of winding and/or twisting. In some cases, the liquid may even be applied to the yarn after winding onto cones, spools, bobbins, or the like or by the so-called "bobbin to bobbin" method. In the case of staple fiber manufacture, the liquid may be applied to the yarn prior to, or after cutting into staple lengths.

The amount of the agent so employed will vary widely depending upon the results desired, the specific nature of the material to which the agent is applied, the use to which the yarn is eventually to be put and other factors. For example, in a given case where a cellulose organic acid ester yarn such as a yarn composed of cellulose acetate, is intended for knitting, about 4 to 25% or more by weight, based on the weight of the dry yarn, may be satisfactory, while if the yarn is intended for weaving, the amount may vary between about 1 and 5%.

Although in the above examples I have referred primarily to yarn treating compositions containing only the conditioning agent and an oil, other ingredients such as solvents, non-solvents, emulsifying agents, blending agents and the like, may be added within the scope of my invention. Likewise, various dyes or other coloring matter may be included in case it is desired to permanently or fugitively tint or dye the material undergoing treatment.

Although I have found it convenient to illustrate my invention by reference to compositions containing specific percentages of the various ingredients, these percentages may vary widely depending upon the particular purpose for which the composition is intended. For example, if it is desired to control the deelectrifying action of the conditioning agent, the amount of the agent may be adjusted as, for example, by reducing the amount of the agent and correspondingly increasing the amount of oil or other ingredient.

While I have described my invention with particular reference to the treatment of yarns composed of organic derivatives of cellulose such as cellulose acetate, the conditioning agents and formulas described herein are applicable to the conditioning of many other types of cellulose derivative yarns such as those composed of or containing cellulose propionate, cellulose butyrate, cellulose acetate propionate, cellulose acetate butyrate, ethyl cellulose, methyl cellulose, benzyl cellulose and others, as well as to the conditioning of silk, wool, cotton, viscose and other natural or artificial materials.

The term "yarn" as used herein and in the claims is to be understood as including a single filament, a plurality of filaments associated into the form of a thread, either of high or low twist, single or multiple threads associated or twisted together, composite threads composed of a mixture of natural and artificial filaments or a composite thread formed by twisting together individual strands of natural or artificial materials, as well as cut staple fibers produced from natural and/or artificial filaments or threads and spun yarn produced from such staple fibers.

As indicated above, the yarn conditioning agents of my invention are exceptionally good solvents for a wide variety of mineral, blown and unblown, drying and semi-drying animal and vegetable oils such as cottonseed, olive, castor, neat's-foot, sperm and other oils. This enables them to be used with any of such oils in making up a variety of yarn treating formulas of varying composition.

The yarn conditioning agents of my invention also have exceptional value as surface-active compounds and as such may be employed as wetting agents, emulsifying and dispersing agents, textile assistants, dye dispersing agents and the like.

The yarn conditioning method and compositions of my invention possess many outstanding advantages. The fundamental and outstanding characteristics of the agents employed in accordance with the invention is their ability to de-electrify yarns, especially those composed of or containing organic derivatives of cellulose such as cellulose acetate and render them amenable to various textile operations, especially operations such as those involved in the manufacture of cut staple fibers, as well as in weaving and knitting. Another outstanding characteristic of these compounds is their exceptional solvent power for a wide variety of mineral, animal, and vegetable

oils and their ability to act as lubricating assistants in conjunction with these oils when applied to such yarns. In addition, due to their solubility in water, they may be readily removed from yarns and fabrics by means of the usual aqueous scour baths.

Of the above compositions I have found those of Example 1, the fifth composition of Example 5, and Example 6 as of outstanding value for the purpose of my invention.

What I claim and desire to secure by Letters Patent of the United States is:

1. The method of eliminating the tendency of yarns, filaments or fibers to accumulate charges of static electricity, which comprises applying thereto prior to any textile operation thereon a composition containing as its essential anti-static component an ester of an alcohol selected from the group consisting of the phosphato, phosphito and sulfato esters of alcohols, said alcohols having the general formula:



wherein R is an organic radical selected from the group consisting of methyl, ethyl, butyl, amyl, hexyl, cyclohexyl, allyl, octyl, lauryl, cetyl, oleyl, hydroxy ethyl, naphthenyl, tetrahydrofurfuryl, decahydronaphthol, triethylene glycol, and monoethyl ether of diethylene glycol, and x is 0 or an integer not over 3, and Z is a mono-valent substituent selected from the group consisting of alkyl, hydroxyl, and aryl.

2. The method of eliminating the tendency of yarns, filaments or fibers composed of or containing organic derivatives of cellulose, to accumulate charges of static electricity, which comprises applying thereto prior to any textile operation thereon a composition containing as its essential anti-static component an ester of an alcohol selected from the group consisting of the phosphato, phosphito and sulfato esters of alcohols, said alcohols having the general formula:



wherein R is an organic radical selected from the group consisting of methyl, ethyl, butyl, amyl, hexyl, cyclohexyl, allyl, octyl, lauryl, cetyl, oleyl, hydroxy ethyl, naphthenyl, tetrahydrofurfuryl, decahydronaphthol, triethylene glycol, and monoethyl ether of diethylene glycol, and x is 0, or an integer not over 3, and Z is a mono-valent substituent selected from the group consisting of alkyl, hydroxyl, and aryl.

3. The method of eliminating the tendency of yarns, filaments or fibers composed of or containing cellulose acetate to accumulate charges of static electricity, which comprises applying thereto prior to any textile operation thereon a composition containing as its essential anti-static component an ester of an alcohol selected from the group consisting of the phosphato, phos-

phito and sulfato esters of alcohols, said alcohols having the general formula:



wherein R is an organic radical selected from the group consisting of methyl, ethyl, butyl, amyl, hexyl, cyclohexyl, allyl, octyl, lauryl, cetyl, oleyl, hydroxy ethyl, naphthyl, tetrahydrofurfuryl, decahydronaphthol, triethylene glycol, and monoethyl ether of diethylene glycol, and x is 0 or an integer not over 3, and Z is a mono-valent substituent selected from the group consisting of alkyl, hydroxyl, and aryl.

4. The method of eliminating the tendency of yarns, filaments or fibers composed of or containing organic derivatives of cellulose to accumulate charges of static electricity, which comprises applying thereto prior to any textile operation thereon a composition containing as its essential anti-static component 2-butyl cyclohexanol sulfate.

5. The method of eliminating the tendency of yarns, filaments or fibers composed of or containing organic derivatives of cellulose to accumulate charges of static electricity, which comprises applying thereto prior to any textile operation thereon a composition containing as its essential anti-static component 2-cetyl cyclohexyl sulfate.

6. The method of eliminating the tendency of yarns, filaments or fibers composed of or containing organic derivatives of cellulose to accumulate charges of static electricity, which comprises applying thereto prior to any textile operation thereon a composition containing as its essential anti-static component 2-amyl cyclohexyl phosphate.

7. Textile yarns having a lessened tendency to accumulate charges of static electricity, said yarns containing an ester of an alcohol selected from the group consisting of the phosphato, phosphito and sulfato esters of alcohols, said alcohols having the general formula:



wherein R is an organic radical selected from the group consisting of methyl, ethyl, butyl, amyl, hexyl, cyclohexyl, allyl, octyl, lauryl, cetyl, oleyl, hydroxy ethyl, naphthyl, tetrahydrofurfuryl, decahydronaphthol, triethylene glycol, and monoethyl ether of diethylene glycol, and x is 0 or an integer not over 3, and Z is a mono-valent substituent selected from the group consisting of alkyl, hydroxyl, and aryl.

10  
1520  
25

30

35

40

45

50

55

60

65

8. Textile yarns composed of or containing organic derivatives of cellulose having a lessened tendency to accumulate charges of static electricity, said yarns containing an ester of an alcohol selected from the group consisting of the phosphato, phosphito and sulfato esters of alcohols, said alcohols having the general formula:



wherein R is an organic radical selected from the group consisting of methyl, ethyl, butyl, amyl, hexyl, cyclohexyl, allyl, octyl, lauryl, cetyl, oleyl, hydroxy ethyl, naphthyl, tetrahydrofurfuryl, decahydronaphthol, triethylene glycol, and monoethyl ether of diethylene glycol, and x is 0 or an integer not over 3, and Z is a mono-valent substituent selected from the group consisting of alkyl, hydroxyl, and aryl.

9. Textile yarns composed of or containing cellulose acetate having a lessened tendency to accumulate charges of static electricity, said yarns containing an ester of an alcohol selected from the group consisting of the phosphato, phosphito and sulfato esters of alcohols, said alcohols having the general formula:



wherein R is an organic radical selected from the group consisting of methyl, ethyl, butyl, amyl, hexyl, cyclohexyl, allyl, octyl, lauryl, cetyl, oleyl, hydroxy ethyl, naphthyl, tetrahydrofurfuryl, decahydronaphthol, triethylene glycol, and monoethyl ether of diethylene glycol, and x is 0 or an integer not over 3, and Z is a mono-valent substituent selected from the group consisting of alkyl, hydroxyl, and aryl.

10. Textile yarns composed of or containing organic derivatives of cellulose having a lessened tendency to accumulate charges of static electricity, said yarns containing 2-butyl cyclohexanol sulfate.

11. Textile yarns composed of or containing organic derivatives of cellulose having a lessened tendency to accumulate charges of static electricity, said yarns containing 2-cetyl cyclohexyl sulfate.

12. Textile yarns composed of or containing organic derivatives of cellulose having a lessened tendency to accumulate charges of static electricity, said yarns containing 2-amyl cyclohexyl phosphate.

JOSEPH B. DICKEY.